

Aug. 18, 1931.

L. G. FIRTH

1,819,365

MOLD

Filed Nov. 2, 1929

Fig. 1.



Fig. 5.



Fig. 2.



INVENTOR

L. Gerald Firth  
by  
Byrne, Stobbs, Penruddick & Blewka  
Attest.

## UNITED STATES PATENT OFFICE

LEWIS GERALD FIRTH, OF PITTSBURGH, PENNSYLVANIA, ASSIGNOR TO FIRTH-STERLING STEEL COMPANY, OF MCKEESPORT, PENNSYLVANIA, A CORPORATION OF PENNSYLVANIA

## MOLD

Application filed November 2, 1929. Serial No. 404,468.

This invention relates to molds for casting metal and to a method whereby metallic bodies may be formed which are substantially free from shrinks, pipes, segregated 5 impurities and gases.

Ingots of metal such as steel ordinarily are cast in vertical molds. These molds usually are provided with hot tops which decrease the tendency towards shrinking and 10 piping by maintaining the top of the ingot hot for a longer time than the remainder of the ingot. The top portion of the ingot, which was the last portion to cool, contains the objectionable defects such as shrinks, 15 pipes and segregated impurities and is usually discarded. For some purposes, however, where it is desired to produce a metallic body which is substantially free from segregated impurities, the method of discarding the upper 20 portion of the ingot does not suffice. The ingot not only cools from the bottom toward the top, but also cools inwardly towards its center; that is, the outside of the ingot in contact with the mold cools first and there is 25 a progressive cooling toward the center so that the last portion in each horizontal plane through the ingot which cools is the center. It is probable that the central 5% to 15% of this cross section cools almost simultaneously; that is, the solidification is progressive inwardly from the sides of the mold up to a 30 central point, after which point more or less simultaneous freezing takes place. It is this central 5% to 15% which contains the greater part of the segregated impurities and 35 gases. Therefore, even if the top portion of the ingot is discarded there is a central core coincident with the longitudinal axis of the ingot which contains some segregated impurities. It is impractical under present 40 practice to discard the whole of that central axis or core which extends from the bottom to the top of the ingot and which contains the steel last to cool in each horizontal plane.

In accordance with my invention, the metal is cast in a mold having a portion provided with insulating material. The portion of the ingot cast adjacent to the insulated portion of the mold accordingly cools more slowly 45 than the rest of the ingot, and this portion

which was the last to cool contains the greater portion of the segregated impurities.

In the preferred embodiment of my invention, a relatively long narrow mold is employed having one end provided with heat insulation. The metal is poured into the mold at the insulated end. The insulation retards the cooling of the metal at one end, but allows relatively rapid cooling at the other end. The segregated impurities collect principally in the insulated end of the mold, leaving the opposite end substantially free from such defects. After cooling, the end of the ingot containing the segregated impurities is separated from the remainder 55 of the ingot.

In the accompanying drawings which illustrate two present preferred embodiments of my invention,

Figure 1 is a side elevation of an ingot 60 mold;

Figure 2 is a horizontal section on the line II-II of Figure 1;

Figure 3 is a vertical side elevation of a 65 modified form of ingot mold, and

Figure 4 is a horizontal section on the line IV-IV of Figure 3.

Referring more particularly to the embodiment shown in Figures 1 and 2, an ingot mold 2 is provided with a hot top 3 having a pouring opening 4 through which metal may be poured into the mold. The mold is provided at its left-hand end, as viewed in Figure 2, with a lining 5 of refractory heat-insulating material. The opposite or right-hand end of the mold, as viewed in Figure 3, has no insulation, but on the contrary the metal in this end of the mold is rapidly cooled by contact with the walls of the mold.

Referring to the embodiment illustrated 70 in Figures 3 and 4, the arrangement differs from that shown in Figures 1 and 2 only in that the mold 2a is made in two parts, 6 and 7, which are secured together by bolts 8. The left-hand end of the mold 2a is provided with 75 a refractory heat-insulating material 5a.

In practicing the invention, the metal is preferably poured through the hot top into the mold, although, if desired, the hot top may be omitted. Insulating material 5 or 100

5a maintains the portion of the ingot which is cast in the left-hand end of the mold hot for a longer time than the remaining portion. The right-hand end of the ingot, which is in contact with the sides and right-hand end 9 of the mold, is rapidly cooled. The impurities and gases segregate and collect at the left-hand end of the ingot mold. The segregated impurities are indicated by the numeral 10.

After the ingot has cooled, the portion 11 which is substantially free from segregated impurities is separated from the portion 12. The portion 11 is thereafter rolled or otherwise worked according to usual practice.

From the above description, it will be seen that in accordance with my method that portion in each horizontal plane through the ingot which was last to cool and which contains segregated impurities and shrinks is discarded and that the remaining portion of the ingot in each horizontal plane is substantially free from such defects. Under ordinary practice heretofore known, the last portion of the ingot to cool in each horizontal plane is in the center of the ingot and for this reason it was impracticable to discard this portion.

In accordance with my invention, the portion of the ingot which is last to cool in each horizontal plane is preferably located at one end of the ingot so that this portion which was last to cool and which contains the segregated impurities and shrinks may be separated from the remaining portion of the ingot which is substantially free from the above defects.

I have illustrated and described two present preferred embodiments of the invention. 40 It is to be understood, however, that the invention may be otherwise embodied or practiced within the scope of the following claims.

I claim:

45 1. A substantially rectangular mold having walls of good heat conducting properties, and a lining of refractory heat insulating material in one end of the mold, said lining covering one end wall and a portion of the adjacent side walls.

50 2. A mold provided with a pouring opening and having a layer of insulating material on the end wall and a portion of the adjoining side walls of the mold adjacent the opening.

55 3. A relatively long narrow ingot mold having a pouring opening adjacent one end thereof, the end and side walls of the mold at the end adjacent the pouring opening having a lining of insulating material which maintains the metal at that end hot for a longer time than the remainder of the metal and causes the segregation and shrinks to form in the insulated end of the mold.

60 4. A mold having walls of good heat con-

ducting properties, one end wall and a portion of the adjoining side walls being lined with insulating material.

5. A mold provided with a pouring opening, the end wall adjacent the pouring opening, and a portion of the adjoining side walls having greater heat insulation properties than the opposite end wall and portions of the side walls adjacent said opposite end wall.

70 6. A vertical ingot mold having walls of good heat conducting properties, one end wall and the adjacent portions of each adjoining side wall being lined with heat insulating material.

75 80 In testimony whereof I have hereunto set my hand.

L. GERALD FIRTH.